

No. 866,883.

PATENTED SEPT. 24, 1907.

A. D. PURTLE & I. E. ROWLAND.  
PROCESS OF MAKING CARBON BLACK.  
APPLICATION FILED DEC. 11, 1906.



WITNESSES:

*C. E. Collier*  
M. E. Collier

*Albert D. Purtle*  
*Irvin E. Rowland* INVENTORS

By *Chas. Snow & Co.*

ATTORNEYS

# UNITED STATES PATENT OFFICE.

ALBERT D. PURTLE AND IRVEN E. ROWLAND, OF SALEM, WEST VIRGINIA.

## PROCESS OF MAKING CARBON-BLACK.

No. 866,883.

Specification of Letters Patent.

Patented Sept. 24, 1907.

Application filed December 11, 1906. Serial No. 347,313.

To all whom it may concern:

Be it known that we, ALBERT D. PURTLE and IRVEN E. ROWLAND, citizens of the United States, residing at Salem, in the county of Harrison and State of West Virginia, have invented a new and useful Process of Making Carbon-Black, of which the following is a specification.

This invention relates to the manufacture of carbon black to be used in the process of making pigments, ink and the like, and has for its principal object to produce the carbon black by a continuous process.

A further object of the invention is to provide a continuous process for the manufacture of a flocculent unctuous carbon black having a slight bluish tinge which may be used for painting or in the manufacture of finer grades of so called India ink.

A still further object of the invention is to provide a process in which a hydro carbon gas under pressure is subjected to the action of heat in a closed retort.

With these and other objects in view, as will more fully hereinafter appear, the invention consists in certain novel features of construction and arrangement of parts, hereinafter fully described, illustrated in the accompanying drawings, and particularly pointed out in the appended claims, it being understood that various changes in the form, proportions, size and minor details of the structure may be made without departing from the spirit or sacrificing any of the advantages of the invention.

The drawing illustrates in vertical section an apparatus for the manufacture of carbon black constructed and arranged in accordance with the invention.

In the drawing 10 indicates a suitable furnace or combustion chamber, within which is arranged a cylindrical retort 11, a number of such retorts being preferably arranged within a single combustion chamber and the opposite ends of each retort projecting beyond the walls of such chamber.

Leading to the retort is a pipe 15 through which gas, preferably natural gas, is forced under pressure, it being found that a pressure of ten pounds secures good results, although both higher and lower pressures have been used in practice. The pipe 15 is provided with a controlling valve 16 through which the gas must pass before it enters the retort, and leading from the pipe is a branch pipe 17, also provided with a controlling valve 18. The branch pipe 17 leads to burner pipe 19 arranged below the retort 11 and provided with perforations for the passage of the jets of gas to be used in heating the retort, provision being made for introducing a suitable quantity of air as by means of a Bunsen-burner air-inlet, indicated at 26.

At the entrance end of the retort is a detachable head 20 having a stuffing box 21 through which passes a rod

22 carrying a scraper 23 which is used for the purpose 55 of forcing the deposited carbon black out of the rear end of the retort from whence it falls through a valved discharge pipe 25 and is conveyed away to the storage or packing room.

In practice the valve of the pipe 25 is closed while 60 the valves 16 and 18 are opened, a sufficient quantity of gas passing through the burner tube to heat the retort to the proper temperature, the retort being preferably heated to a bright cherry red or approximately eight hundred degrees centigrade. The carbon of the gas 65 under pressure entering the retort is deposited within the retort in the form of carbon black, and at frequent intervals the scraper 23 is forced through the retort in order to convey away the carbon black from the heat zone before any deterioration from burning can occur, 70 the valve in the discharge pipe being open at intervals to permit the accumulated carbon black to discharge.

The process is to all intents and purposes a continuous one in that it is not necessary to stop operations except momentarily to open the valve of the discharge pipe, and it is never necessary to allow the retort to cool for the removal of the product. 75

We claim:

1. The process of producing carbon black from a hydro-carbon gas which consists in heating the gas in a closed retort to such a degree as to decompose the gas and cause the carbon to be deposited on the interior walls of the retort in a flocculent condition, and then removing the carbon while still in the flocculent state and without cooling 80 the retort.

2. The process of producing carbon black from a hydro-carbon gas consisting in subjecting the gas under pressure in a closed retort to a heat of about 800 degrees centigrade until the carbon is deposited on the interior walls of the 85 retort in a flocculent condition, and then removing the carbon from the retort while still in the flocculent state.

3. The process of producing carbon black from a hydro-carbon gas consisting in continuously introducing the gas under pressure into a closed retort heated to a temperature sufficient to cause the deposition of the carbon of the gas in a flocculent state upon the interior walls of the retort, and then removing the deposited carbon from time to time while still in the flocculent state and without reducing the heat of the retort. 95

4. The process of producing carbon black from a hydro-carbon gas consisting in subjecting the gas under pressure in a closed retort to the action of heat until the carbon is separated therefrom and deposited in a flocculent condition in the retort, and then removing the deposited carbon 100 while still in the flocculent state, from the heat zone.

In testimony that we claim the foregoing as our own, we have hereto affixed our signatures in the presence of two witnesses.

ALBERT D. PURTLE.  
IRVEN E. ROWLAND.

Witnesses:

OSCAR C. WILT,  
O. F. MORRISON.